

# United States Patent

Stephan et al.

[15] 3,635,776

[45] Jan. 18, 1972

[54] **PRODUCTION OF BONDED  
NONWOVENS BY THE WET METHOD**

[72] Inventors: Rudolf Stephan, Ludwigshafen; Gerhard Welzel, Mannheim; Hans Reinhard, Limburgerhof; Hans-Ulrich Frank, Ludwigshafen, all of Germany

[73] Assignee: Badische Anilin- & Soda-Fabrik Aktiengesellschaft, Ludwigshafen, Rhine, Germany

[22] Filed: June 27, 1969

[21] Appl. No.: 837,312

[30] **Foreign Application Priority Data**

June 29, 1968 Germany ..... P 17 69 700.6

[52] U.S. Cl..... 156/315, 156/181, 156/331,  
156/332, 156/333, 156/334

[51] Int. Cl..... C09j 5/04

[58] Field of Search..... 156/181, 281, 314, 331, 315,  
156/332, 333, 334

[56]

**References Cited**

**UNITED STATES PATENTS**

2,927,051 3/1960 Buckwalter et al. .... 156/314 X  
3,510,390 5/1970 Bjorksten et al. .... 156/314 X

*Primary Examiner*—Carl D. Quarforth

*Assistant Examiner*—Stephen J. Lechert, Jr.

*Attorney*—Johnston, Root, O'Keeffe, Keil, Thompson & Shurtleff

[57]

**ABSTRACT**

Bonded nonwovens can be produced with particular advantage by the wet method by treating the textile fibers prior to the addition of the binder polymers with water-soluble cationic polycondensation products which have been prepared from carbamides, formaldehyde, dicyanodiamide and salts of ammonia or of amines.

8 Claims, No Drawings

## PRODUCTION OF BONDED NONWOVENS BY THE WET METHOD

This invention relates to a process for the production of bonded nonwovens by the wet method.

In the wet method for the production of bonded nonwovens natural or synthetic textile fibers are suspended in an aqueous medium and a bonding agent is added. The aqueous medium is then separated on a machine substantially resembling known paper machines and the resultant web is generally dried at elevated temperature.

Fibers known as binder fibers, for example of polyvinyl acetate or of cellulose loaded with polyacrylates, are often used as binders for bonding nonwovens. The webs of fibrous material thus acquire adequate wet tear resistance to enable them to be removed from the wire of the machine. When drying and heating is carried out, the polyvinyl acetate fibers or the polyacrylates are softened so that the textile fibers are bonded together. The tear resistance of bonded nonwovens obtained by these known methods is however inadequate. For this reason, the bonded nonwovens are often additionally impregnated with a plastics dispersion or solution. However, the handle of nonwovens prepared in this way is usually hard and similar to that of paper.

It is furthermore known from British Pat. No. 1,071,136 that paper and nonwovens can be prepared from fibers which have been treated successively with melamine resins or urea resins and an aqueous dispersion of a plasticized thermoplastic. If bonded nonwovens are prepared from such pretreated plastics by the wet method, products are obtained however from which the plasticizer can easily migrate. As a result, the handle becomes less good and in some cases the material becomes more prone to soiling.

The object of the present invention is an improvement in the known method for the production of bonded nonwovens by the wet process in which conventional binder polymers can be used and in which nonwovens having particularly high initial tear resistance and particularly high tensile strength are obtained.

We have now found that the production of bonded nonwovens by the wet method by suspending textile fibers in an aqueous medium, precipitating a binder polymer dispersed in the aqueous medium onto the fibers, separating the aqueous medium and drying the nonwoven at elevated temperature, can be advantageously carried out by treating the textile fibers with water-soluble cationic polycondensation products which have been prepared from a carbamide, formaldehyde, dicyandiamide and a salt of ammonia or of an amine.

Suitable water-soluble cationic polycondensation products of a carbamide, formaldehyde, dicyandiamide and a salt of ammonia or an amine are obtainable for example according to the process of German Pat. No. 1,078,768 according to which condensation products having a uniform degree of condensation from formaldehyde and a carbamide such as urea, alkylureas, acetylenedurea with dicyandiamide and with a salt of ammonia or an aliphatic amine are condensed with an inorganic or strong organic acid and if desired with a further amount of formaldehyde; hexamethylene tetramine may also be cocondensed. Instead of using condensation products having a uniform degree of condensation from formaldehyde with carbamides, similar products having a nonuniform degree of condensation may be used.

Examples of particularly suitable alkylureas for the production of the cationic polycondensation products are N-alkylureas and N,N'-dialkylureas whose alkyl groups usually have one to three carbon atoms, such as N-methylurea, N,N'-dimethylurea, N-ethylurea, N,N'-diethylurea, N-n-propylurea and N,N'-diisopropylurea. Alkylureas of the said type which contain more than three, for example from four to six, carbon atoms in their alkyl groups are also suitable. Suitable carbamides of the said type generally contain one to seven, preferably one to four, carbon atoms and urea is the preferred carbamide. Suitable aliphatic amines for formation of salts are particularly N-monoalkyl-amines, N,N-dialkylamines, N-alkylolamines, N,N-dialkylolamines and N,N,N-trialkylolamines

whose alkyl radicals usually contain from one to three, particularly one or two, carbon atoms. Specific examples are methylamine, ethylamine, propylamine, isopropylamine, dimethylamine, diethylamine, ethanolamine, N,N-diethanolamine and triethanolamine. Examples of salts of ammonia are ammonium chloride, bromide, phosphate, formate and chloroacetate.

In the production of the condensation products by condensation in alkaline or acid medium for example according to the method known from German Pat. No. 1,078,768, generally from two to four moles of formaldehyde are used for each mole of carbamide of the said type in the first stage.

Low molecular weight compounds can be used as starting material for the second stage of the process. These may be (when urea has been condensed with formaldehyde) compounds such as dimethylolurea, trimethylolurea and tetramethylolurea. Higher molecular weight products which are still soluble in water and which have been obtained by further condensation may however also be used. Condensation products which are already water repellent and which have been obtained by condensation at pH values of less than 7.0 are also suitable.

Conversion of the neutral condensation products of the first stage into cationic products with dicyandiamide, ammonium salts or amine salts with or without an additional amount of formaldehyde may be carried out by several methods. For example the components of the second stage may be added immediately to the reaction mixture of the first stage. The reaction mixture of the first stage may be concentrated, for example by vacuum evaporation, prior to further processing. Condensation in the second stage is carried out in the acid range. The condensation temperature may be from 50° to 100° C.; the reaction period may be from 15 minutes to 2 hours or more. Cationic condensation products having a definite degree of condensation may easily be obtained in a reproducible manner by selection of the appropriate reaction conditions; the degree of condensation may be regulated by reference to the viscosity or the turbidity point (cf. example 2) or the pH value.

As regards the amounts of the reaction components the following may be said: calculated on a condensation product of the first stage obtained from 1 mole of carbamide, particularly urea, about 0.5 to 2 moles of dicyandiamide, 1 to 3 moles of ammonium or amine salt or a mixture of such salts and in both stages together from 3 to 6 moles of formaldehyde may be used. The formaldehyde may be used in the form of the commercial aqueous solution of 30 by weight or 40 by volume strength; it may however also be added as paraformaldehyde to the aqueous solution of the carbamide.

When using ammonium or amine salts of hydrochloric acid, products are obtained which are soluble in water in all proportions provided that at least as many moles of formaldehyde have been cocondensed as there are moles of carbamide, dicyandiamide and ammonium or amine salt present. On the other hand sulfates or, generally speaking, anions having a greater ion radius give condensation products having a limited solubility in water.

The solubility in water of products which are not dilutable in every ratio with water or the stability of condensation products which are completely soluble in water to precipitants, for example nitrate or sulfate ions, can be increased by introducing by condensation in the second process stage about one-sixth to one-third of a mole of hexamethylenetetramine. This additional measure is of special advantage when ammonium salts having anions of great radius, such as  $\text{NO}_3^{(-)}$ ,  $\text{SO}_4^{(--)}$  and  $\text{I}^{(-)}$ , have been used in the condensation, because the water-solubility of such condensation products is generally less than that of products obtained under otherwise the same conditions with for example ammonium chloride and ammonium bromide. When more than 1 mole of formaldehyde is used in the first stage of the condensation per mole of carbamide and the moles of dicyandiamide and ammonium or amine salt to be added to the second stage, the excess moles of formal-

dehyd<sup>e</sup>e can be reacted by adding an appropriate amount of ammonia to form hexamethylenetetramine and the addition of hexamethylene tetramine can be dispensed with.

Polymers suitable for the preparation of bonded nonwovens, which are generally in the form of their aqueous dispersions, are suitable as binder polymers. Aqueous dispersions which contain from 40 to 60 percent by weight of acrylic ester and/or methacrylic ester polymers having carboxyl groups are particularly suitable. These polyacrylates are usually derived from esters of acrylic or methacrylic acid with alkanols containing from one to 12, particularly from one to eight, carbon atoms, which often form the major component of the copolymers. Such polyacrylates generally contain (as monomers having carboxyl groups) from 1 to 10 percent by weight of polymerized units of  $\alpha$ ,  $\beta$ -olefinically unsaturated monocarboxylic and/or dicarboxylic acids which preferably contain from three to five carbon atoms. The proportion of such olefinically unsaturated carboxylic acids in the copolymers is preferably from 2 to 2 percent by weight with reference to the copolymer. Acrylic and methacrylic acid are particularly suitable; crotonic acid, maleic acid, fumaric acid and itaconic acid are also suitable. The polyacrylates may additionally contain polymerized units of further olefinically unsaturated monomers, for example vinyl-aromatic compounds, such as styrene, vinyl halides or vinylidene halides, such as vinyl chloride and vinylidene chloride, acrylonitrile, methacrylonitrile and/or vinyl esters of saturated carboxylic acids containing from two to 18, particularly two to three, carbon atoms, particularly vinyl acetate and vinyl propionate but also vinyl laurate, vinyl stearate and vinyl pivalate, and also (usually in amounts of from 1 to 10 percent, particularly from 2 to 7 percent, by weight with reference of the copolymer) of amides of  $\alpha$ ,  $\beta$ -olefinically unsaturated monocarboxylic and/or dicarboxylic acids usually containing from three to five carbon atoms or their derivatives, particularly acrylamide, methacrylamide, N-methylolacrylamide, N-methylolmethacrylamide, N-methoxymethylmethacrylamide, N-n-butoxymethylmethacrylamide, N-acetoxymethylacrylamide and N-acetoxymethylmethacrylamide, and vinyl-sulfonic acids or their salts. The aqueous dispersions of such polyacrylates may contain conventional anionic and/or nonionic emulsifiers with or without small amounts of protective colloids.

Other suitable binder polymers are the aqueous dispersions (conventionally used for the purpose) based on polymers of vinyl chloride and/or vinylidene chloride, based on butadiene-styrene copolymers or butadiene-acrylonitrile copolymers and/or based on vinyl ester polymers, for example polymers of vinyl acetate or vinyl propionate, which may contain conventional anionic or nonionic emulsifiers with or without protective colloids.

Generally from 1 to 10 percent, preferably from 3 to 6 percent, by weight of water-soluble cationic polycondensation products and from 10 to 60 percent, preferably from 30 to 50 percent, by weight of binder polymer (in each case calculated as solids and with reference to the amount of textile fibers) are used in the new process.

The amount of textile fibers (with reference to the amount of water) is usually from 0.5 to 3 percent, preferably from 0.7 to 1.5 percent, by weight, the fibers preferably having a length of from 5 to 30 mm. The textile fibers may consist for example of cellulose or cellulose derivatives, synthetic polyamides such as polycaprolactam or polyhexamethylene adipamide, saturated polyesters such as polyethylene glycol terephthalate, or polyacrylonitrile.

In the new process the synthetic fibers may be pretreated with the water-soluble cationic polycondensation products in aqueous suspension and used in the process according to this invention, if desired after drying. The pretreated fibers are then suspended in the aqueous medium and then an aqueous dispersion of the binder polymer is added, generally while stirring. When the binder polymer has been precipitated onto the fibers, the material can be fed to the wire section of a web-forming machine, for example an inclined-wire machine, and

processed by suction or pressing in the conventional manner. The fibers loaded with the binder polymer are generally arranged as a thin sheet material during separation of the aqueous medium. The web can then be lifted off from the wire in the conventional way and dried at elevated temperature which is usually from 60° to 150° C., preferably from 80° to 130° C.

According to an advantageous embodiment of the process, a suspension of the textile fibers may have added to it first an aqueous usually from 5 to 15 percent and preferably from 8 to 10 percent solution of the cationic polycondensation product and simultaneously or some minutes later an aqueous dispersion of the binder polymer. Separation of the aqueous medium and drying of the web may be carried out in the conventional manner.

15 It is advantageous in the new process to add a resin soap to the aqueous suspension of textile fibers in addition to the water-soluble polycondensation product and the binder polymer.

20 The new process gives bonded nonwovens which as compared with other nonwovens prepared by the wet method are distinguished by particularly great initial tear resistance, particularly high tensile strength and by a soft textile handle.

25 Additives conventionally used for finishing textiles and/or paper may be used in the conventional ways and if desired added to the aqueous medium in the new process, provided they are compatible with the other additives.

30 The invention is illustrated by the following examples, in which parts and percentages are by weight.

#### EXAMPLE 1

35 Twenty-five kilograms of a mixture of polycaprolactam fibers of which half have a length of 8 mm. and the other half have a length of 12 mm. is suspended in 2.5 m.<sup>3</sup> of water with an addition of 250 g. of an oxyethylated fatty alcohol. While stirring, a solution of 1,500 g. of a water-soluble cationic polycondensation product prepared as described in example 1 of German Pat No. 1,078,768 from 1 mole of urea, 1 mole of dicyandiamide, 3 moles of formaldehyde and 1 mole of ammonium chloride in 5 liters of water, and a solution of 250 g. or resin soap in 2.25 liters of water and 20.5 kg. of a 50 percent aqueous dispersion of a copolymer of 93 parts of n-butyl acrylate, 1 part of acrylic acid, 3 parts of N-methylolmethacrylamide and 3 parts of acrylonitrile are added. The whole is stirred for another 10 to 20 minutes and the aqueous suspension is introduced into a web-forming machine. The water is separated and the web is lifted off and dried at 120° C. A nonwoven is obtained which in the dry condition has a tensile strength of 120 kg./cm.<sup>2</sup> measured according to DIN 53,112. The nonwoven has a soft textile handle and is suitable for the production of nonwoven clothing, disposable articles, disposable bed linens and the like.

40 45 50 55 Twenty-five kilograms of a mixture of equal parts of cotton linters and wool flock may be used instead of the polycaprolactam fibers.

#### EXAMPLE 2

60 Twenty-five kilograms of a mixture of equal parts of polycaprolactam fibers (1.5 denier/10 mm.), viscose rayon fibers (1.5 denier/10 mm.) and beech sulfite cellulose is suspended in 2.5 m.<sup>3</sup> of water. A solution of 2,000 g. of the water-soluble cationic polycondensation product specified in example 1 in 10 liters of water is added while stirring. It is allowed to go onto the fibers for 10 to 15 minutes. Then a mixture of a solution of 750 g. resin soap in 10 liters of water and 22.5 kg. of a 50 percent aqueous dispersion of a copolymer of 93 parts of n-butyl acrylate, 1 part of acrylic acid, 3 parts of N-methylolmethacrylamide and 3 parts of acrylonitrile is added to the suspension of fibers. After 10 to 20 minutes, the aqueous suspension of the fibers loaded with plastic is introduced into the web-forming machine. The water is separated and the web is lifted off from the wire and dried at 120° C. A nonwoven is obtained which in the dry condition has a tensile strength of 100 kg./cm.<sup>2</sup> measured according to DIN 53,112.

The nonwoven has a soft textile handle and is suitable for the production of nonwoven clothing, furnishings, disposable articles and the like.

We claim:

1. In a wet method for production of nonwoven textile fiber articles by suspending textile fibers in aqueous medium, depositing on the fibers a binder polymer dispersed in the aqueous medium, separating the aqueous medium from the fibers loaded with the binder polymer and drying the resultant web at elevated temperature, the improvement which comprises treating the textile fibers, prior to the addition of the binder polymer, with a water-soluble cationic polycondensation product, which has been prepared from a carbamide containing from one to seven carbon atoms, formaldehyde, dicyandiamide and a salt of ammonia or an amine, said water soluble cationic polycondensation product having been produced by reacting (a) a water soluble condensation product of formaldehyde and said carbamide in a mole ratio of 1.2 to 4, respectively with (b) 0.5 to 2 moles of dicyandiamide, and (c) at least one of (a') 1 to 3 moles of an N-monoalkyl amine, an N,N-dialkylamine, an N-alkylolamine, an N,N-dialkylolamine or an N,N,N-trialkylolamine wherein the alkyl or alkylol groups thereof contain one to three carbon atoms or (b') 1 to 3 moles of an ammonium salt at 50°-100° C., in acidic aqueous medium, said moles being based upon 1 mole

25

of said carbamide in said water soluble condensation product, and the total moles of formaldehyde used in the preparation of said cationic polycondensation product being in the range of 3 to 6 moles per 1 mole of said carbamide in said condensation product (a).

2. In a method as claimed in claim 1, said carbamide having one to four carbon atoms.

3. In a method as claimed in claim 1, said carbamide being urea.

4. In a method as claimed in claim 1, said carbamide being urea, N-alkylurea or N,N-dialkylurea, said alkyl groups having one to six carbon atoms.

5. In a method as claimed in claim 1, said water soluble condensation product (a) being dimethylolurea, trimethylolurea or tetramethylolurea

6. In a method as claimed in claim 1, the anions of said salts being chloride, bromide, iodide, phosphate, formate, chloroacetate, sulfate or nitrate.

7. In a method as claimed in claim 1, and reacting with (a) and (b) about one-sixth to one-third mole of hexamethylenetetramine.

8. In a method as claimed in claim 1, wherein the amount of said water soluble cationic polycondensation product is 1-10 percent by weight, on a solid basis, of said textile fibers.

\* \* \* \* \*

30

35

40

45

50

55

60

65

70

75

UNITED STATES PATENT OFFICE  
CERTIFICATE OF CORRECTION

Patent No. 3,635,776

Dated January 18, 1972

Inventor(s) Rudolf Stephan et al

It is certified that error appears in the above-identified patent and that said Letters Patent are hereby corrected as shown below:

Column 2, line 48, "30 by weight or 40" should read -- 30% by weight or 40% --.

Column 4, line 41, "or" should read -- of --.

Column 5, line 19, "or" should read -- of --.

Signed and sealed this 6th day of June 1972.

(SEAL)

Attest:

EDWARD M. FLETCHER, JR.  
Attesting Officer

ROBERT GOTTSCHALK  
Commissioner of Patents